

Aug. 11, 1925.

1,549,312

D. D. JACKSON ET AL  
PROCESS OF DESULPHURIZING IRON AND STEEL AND A COMPOSITION  
OF MATTER FOR USE IN SAID PROCESS  
Filed Feb. 22, 1922

Fig. 1.



Fig. 2.



INVENTORS:

Daniel D. Jackson  
Joseph D. Sears  
Frederick Conlin

By Attorneys,

*Frazer, Park & Meyer*

## UNITED STATES PATENT OFFICE.

DANIEL D. JACKSON, OF BROOKLYN, NEW YORK, JOSEPH D. SEARS, OF BLOOMFIELD, AND FREDERICK CONLIN, OF WESTFIELD, NEW JERSEY, ASSIGNORS TO SAID JACKSON, SAID SEARS, AND JOHN T. PRATT, OF NEW YORK, N. Y., AS JOINT TRUSTEES.

PROCESS OF DESULPHURIZING IRON AND STEEL AND A COMPOSITION OF MATTER FOR USE IN SAID PROCESS.

Application filed February 22, 1922. Serial No. 538,423.

*To all whom it may concern:*

Be it known that we, DANIEL D. JACKSON, residing in the borough of Brooklyn, city and State of New York, JOSEPH D. SEARS, residing in Bloomfield, county of Essex, and State of New Jersey, and FREDERICK CONLIN, residing in Westfield, county of Union, State of New Jersey, citizens of the United States of America, have invented certain new and useful Improvements in Processes of Desulphurizing Iron and Steel and a Composition of Matter for Use in Said Processes, of which the following is a specification.

15 This invention relates to a process of treating iron, steel, ferro-alloys and copper, for reducing or eliminating the sulphur content thereof, and to a composition of matter for use in such process, and aims to provide

20 improvements therein.

The invention provides an improved and highly effective process of reducing or eliminating the sulphur content in iron, steel, ferro-alloys and copper. It further provides a process which is very simply and readily carried out in connection with present operating equipment in general use for producing iron, steel, etc.

25 The invention further provides a process using a class of reagents which are in abundant supply in the market.

The invention further provides a composition of matter, which is useful in the above-mentioned process and which may be put up in a form convenient for use and safe for handling.

30 A specific application of the process and a form in which the composition of matter may be embodied are illustrated in Figures 1 and 2 respectively of the accompanying drawing.

According to our discovery and researches, sulphur, found as an impurity in iron, steel, etc., can be virtually eliminated, or its content in iron, steel, etc., substantially reduced by treating the molten metal containing the sulphur with certain mixtures of alkali-metal compounds, which unite or combine with the sulphur compound of the iron. A

number of alkali-metal compounds have 50 been found to give good results in reducing the sulphur content of iron and steel. Among these substances may be mentioned sodium hydroxid, sodium carbonate, potassium carbonate, potassium hydroxid, and 55 sodium or potassium silicate together with one or more of the preceding.

Our researches and discoveries have also shown that the sodium compounds, in combination with sodium silicate, give a decidedly superior desulphurizing action.

Our researches and discoveries have also shown that mixtures of alkali-metal hydroxids and carbonates indiscriminately with other substances, instances of which 65 are found in prior art patents, do not have an action which can be regarded as of significant or technical importance.

It is not intended to be indicated herein, however, that the alkali-metal compounds, 70 or their mixtures with alkali-metal silicates, as set forth herein, may not be used together with other substances which do not destroy or materially disadvantageously affect the desulphurizing action of said reagents.

Using sodium hydroxid as the reagent, the reaction upon the sulphur in the metal would probably be—



80 The alkali-metal reagent is brought into contact with the molten iron, steel, etc., in any suitable or known manner practiced in 85 metallurgy, but is conveniently placed or dumped onto the surface of the metal contained in an ordinary ladle, crucible, converter, hearth, or the like. Any overlying slag, so far as possible, is removed from the 90 surface of the molten metal. A complete covering of the surface of the metal with the desulphurizing material will give the greatest efficiency. The heat of the metal will dissociate the sodium hydroxid, which 95 will break up into sodium oxid and water vapor which will be evolved. The sodium hydroxid will be melted to a fluid consis-

tency by the heat of the molten metal, and will flow over the surface thereof, and the sulphur in the mass of the iron, steel, etc., will be brought by convection currents in the mass into contact with the liquid layer of the sodium hydroxid on the surface thereof, thereby reacting with the sodium oxide to form sodium sulphide, and probably some one or more oxy-sulphur sodium compounds, which enter the slag produced by the treatment.

In the drawing, Fig. 1 the molten metal (designated by reference letter A) is illustrated as being contained in a ladle B. C designates the surface layer of liquid sodium hydroxid.

In experiments on iron, using a mixture of sodium hydroxid and sodium carbonate (equal parts) as the desulphurizing reagent, spread out as a liquid layer on the surface of the molten iron, a reduction as high as 67% of the sulphur contained in the iron has been obtained, at a single treatment, viz., a reduction from .146% S. to .048% S.

It has been further discovered that a better result in reducing the sulphur content of iron, steel, etc., by the use of the reagents hereinbefore mentioned, may be obtained by using said reagents concurrently with an alkali-metal silicate. The alkali-metal reagent and the alkali-metal silicate are conveniently mixed, and the mixture used in the same manner as the use of the alkali-metal reagent has been described. For convenience in handling, the two or mixed reagents are preferably fused into cakes of a regular size, and for comfort and safety in handling, where one of the ingredients may be caustic, and for preserving the condition of the mixture where one of the ingredients may be hygroscopic, the mixture may be covered in any suitable manner, as by a box, or by a coating of paraffine.

In the drawing, Fig. 2, which illustrates a form of the composition of matter comprising the alkali-metal reagent and the alkali-metal silicate, the letter M designates a cake consisting of a fused mixture of said ingredients, and O designates a coating of paraffine wax covering said cake.

With a mixture of sodium hydroxid and sodium silicate (solid water glass) spread out as a liquid layer on the surface of the molten metal, the sulphur content of iron has been reduced as much as 97% at a single treatment, viz., a reduction from .114% S. to .004% S. A mixture of from 85-95% sodium hydroxid to from 5-15% sodium silicate has given best results in use, the highest reduction of sulphur having been obtained with a mixture of 90% sodium hydroxid and 10% sodium silicate (water glass— $\text{Na}_2\text{O} \cdot 4\text{SiO}_2$ ).

In experiments upon iron, using a mixture of sodium carbonate, and sodium sili-

cate spread out as a liquid layer on the surface of the molten metal, the sulphur content of the iron has been reduced as much as 68% at a single treatment, viz., a reduction from .158% S. to .05% S.

In experiments upon iron, using a mixture of sodium hydroxid, sodium carbonate, and sodium silicate in the proportions of 90% sodium hydroxid, and sodium carbonate, and 10% sodium silicate, as the desulphurizing reagent spread out as a liquid layer on the surface of the molten iron, a reduction as high as 75% has been obtained, at a single treatment.

With a mixture of sodium hydroxid (90%) and sodium silicate (10%) used on copper (Lake copper) the sulphur content has been reduced as much as 91% at a single treatment, viz., a reduction from .117% S. to .0096% S.

Usually from 10 to 25 pounds of this mixture to a ton of iron is used, depending on the sulphur content and the amount of sulphur desired to be removed. Where the carbonate is used in the place of the hydroxid, or where potassium is used in the place of sodium, the amount to be used may be calculated on the basis of the  $\text{Na}_2\text{O}$  content of the sodium hydroxid.

Corresponding results in foundry practice have been obtained by using the above-mentioned reagents and mixtures thereof with silicates (water glass).

The alkali-metal silicate when used alone will act to reduce the sulphur content of iron, steel, etc., but this per cent. of reduction is small as compared with sodium hydroxid and sodium carbonate, showing about a 14% reduction.

The conjoint use of the alkali-metal silicate (water glass) with another alkali-metal reagent such as sodium hydroxid or carbonate, in the proportions previously designated, gives the best results, as the sulphur reduction in such case is superior to that obtained by any of the alkali-metal reagents alone.

The mixture of alkali-metal hydroxid and alkali-metal carbonate is less volatile when heated on the molten bath than hydroxid alone, produces a less watery layer or slag on the surface of the metal than hydroxid alone, and melts more quickly than carbonate alone. The alkali-metal silicate is used mainly as a binder of the other ingredient or ingredients of the mixture and to thereby promote the quick melting of the mixture.

It is to be understood that the carbonate beside reducing the volatility of the hydroxid, has other beneficial properties such as reducing the tendency of the hydroxid to act on the silicon in the iron, and that the silicate also has other properties, such as reducing the volatility of the hydroxid.

Where the alkali-metal reagent, either

alone or associated with an alkali-metal silicate, is used with other substances which prevent the reagent melting to a thin or fluid consistency, the desulphurizing action 5 has been found to be much inferior to what it is when the reagent is at a thin or fluid consistency.

The process may be carried out by various other procedures than that specifically described. 10

Claims to the mixture of sodium hydroxid and sodium carbonate, and to the fused mixture thereof, and to the process of desulphurizing with this mixture, are contained 15 in our copending application Serial No. 631,925, filed April 13, 1923.

What is claimed is:—

1. A process of treating iron, steel, ferro-alloys, and copper for diminishing or eliminating the sulphur content thereof, comprising treating the molten metal with a mixture of alkali-metal hydroxid and alkali-metal carbonate, the carbonate being present in an amount to reduce the volatilization of the hydroxid. 20

2. A process according to claim 1 in which an alkali-metal silicate is contained in the mixture of hydroxid and carbonate, the silicate binding the other ingredients of the 30 mixture prior to melting.

3. A process of treating iron, steel, ferro-alloys, and copper for diminishing or eliminating the sulphur content thereof, comprising treating the molten metal with a mixture of an alkali-metal silicate, and at least one of the following: alkali-metal hydroxid, alkali-metal carbonate; said silicate binding the other ingredients of the mixture prior to melting. 35

4. A process according to claim 3, further characterized by the silicate being present in the proportion of 5-15% and the alkali-metal hydroxid, or carbonate, or mixture of hydroxid and carbonate, from 85-95%. 40

45 5. A process according to claim 3, further characterized by the silicate being present in the proportion of substantially 10%, and

the alkali-metal hydroxid, or carbonate, or mixture of hydroxid and carbonate, 90%.

6. A process according to claim 1, further 50 characterized by the ingredients being previously fused.

7. A process according to claim 3, further characterized by the ingredients being previously fused. 55

8. A composition of matter for use in desulphurizing iron, steel, ferro-alloys, and copper, consisting of alkali-metal hydroxid and alkali-metal carbonate, the carbonate being present in an amount to reduce the 60 volatilization of the hydroxid at the temperatures of molten metal.

9. A composition of matter for use in desulphurizing iron, steel, ferro-alloys, and copper, consisting of an alkali-metal silicate 65 and at least one of the following: alkali-metal hydroxid, alkali-metal carbonate, the silicate binding the other ingredients of the mixture.

10. A composition of matter according to 70 claim 9, further characterized by the alkali-metal silicate being representatively in the proportion of 5 to 15% and the alkali-metal hydroxid, or carbonate, or mixture, from 85 to 95%.

11. A composition of matter according to 75 claim 9, further characterized by the alkali-metal silicate being substantially in the proportion of 10% and the alkali-metal hydroxid, or carbonate, or mixture, 90%. 80

12. A composition of matter according to claim 8, further characterized by including an air-excluding surface covering.

13. A composition of matter according to 85 claim 9, further characterized by including an air-excluding surface covering.

14. A composition of matter according to claim 9, further characterized by the silicate being water-glass.

In witness whereof, we have hereunto 90 signed our names.

DANIEL D. JACKSON.  
JOSEPH D. SEARS.  
FREDERICK CONLIN.